

May 17, 1960

H. C. YUTZY ET AL

2,937,086

MULTILAYER REVERSAL COLOR MATERIAL

Filed July 26, 1955



HENRY C. YUTZY  
JOHN H. VAN CAMPEN  
INVENTORS

BY *Daniel I. Mayne*  
*P. Frank Smith*  
ATTORNEYS

# United States Patent Office

2,937,086

Patented May 17, 1960

1

2,937,086

## MULTILAYER REVERSAL COLOR MATERIAL

Henry C. Yutzy and John H. Van Campen, Rochester, N.Y., assignors to Eastman Kodak Company, Rochester, N.Y., a corporation of New Jersey

Application July 26, 1955, Serial No. 524,362

2 Claims. (Cl. 96—74)

This invention relates to photography and particularly to a multilayer reversal color material.

Meeussen and Bellay U.S. Patent 2,673,800 describes a reversal color material in which differently-sensitive silver halide emulsion layers containing both non-diffusing couplers capable of coupling with the oxidation product of primary aromatic amino developing agents and development nuclei, are separated from each other by barrier layers. These barrier layers contain substances which check the diffusion of silver salts, such as colloidal silver, silver sulfide and fogged silver halide emulsion. The emulsion layers are exposed and developed in a black and white negative developer, then in a color developer of the p-phenylenediamine type containing a silver halide solvent. The color developer forms positive dye images in the emulsion layers, and the barrier layers prevent diffusion of the silver salts dissolved by the color developing solution, into neighboring emulsion layers.

The Meeussen and Bellay material has the disadvantage that the barrier layers increase the number of coatings and therefore increase the cost and complexity of the material.

It is therefore an object of the present invention to provide an improved multilayer reversal color material. A further object is to provide a multilayer material developed by the solvent transfer process but not requiring barrier layers or interlayers. Other objects will be apparent from the following description of our invention.

These objects are accomplished according to our invention by incorporating in the emulsion layers a non-diffusing coupler capable of reacting with the oxidation product of primary aromatic amino developing agents, a nucleating agent for precipitating dissolved silver salts, and a non-diffusing reducing agent or acceptor for oxidized developer.

In the accompanying drawing the single figure is a sectional view of a sensitive material constructed according to our invention.

Our sensitive material preferably has three silver halide emulsions each sensitive to one of the three primary spectral regions, although only two sensitive layers may be employed. If three sensitive layers are used, the blue-sensitive emulsion is preferably a fast gelatino-silver chlorobromide emulsion, and the green-sensitive and red-sensitive emulsions are preferably slow, optically-sensitized gelatino-silver chlorobromide emulsions. Such coatings require no filter for blue light, and may be coated on the support in any order, that is, with the blue-sensitive layer either outermost or adjacent the support. If faster negative emulsions are used and the blue-sensitive layer is coated outermost, a filter layer of the type described in Saunders et al. U.S. application Serial No. 476,066, Patent No. 2,756,149, may be employed.

The emulsion layers contain non-diffusing coupler compounds such as those described in Salminen and Weissberger U.S. Patent 2,423,730, Porter and Weissberger U.S. Patent 2,369,489, Loria, Weissberger and Vittum

2

U.S. Patent 2,600,788, and Weissberger U.S. Patent 2,298,443. Suitable couplers are, for example:

- 2 - [α - (4' - tert. - amylphenoxy) - n - butyrylamino] - 5- 5 methyl-1-phenol
- 2 - [4''(3' - tert. - amylphenoxy - benzamido) - (- benzamido)]-4-chloro-5-methyl-1-phenol
- 2 - (2',4' - di - tert. - amylphenoxyacetamino) - 4,6 - di-chloro-5-methylphenol
- 10 1 - [p - (p' - tert.butyphenoxy) - phenyl] - 3 - [α - (p- tert.butyphenoxy)propionylamino]-5-pyrazolone
- 1 (p - [p' - tert.butyphenoxy] - phenyl) - 3 - (p - [α - {p' - tert.butyphenoxy} - propionylamino] - benzoyl-amino-5-pyrazolone)
- 15 1 - (2',4',6' - trichlorophenyl) - 3 - [3'' - (2'',4'' - di- tert.amylphenoxyacetamido)-benzamido]-5-pyrazolone
- N - (4 - benzoylacetaminobenzenesulfonyl) - N - (γ- phenylpropyl)-p-toluidine
- N - (p - benzoylacetaminobenzenesulphonyl) - N - (γ- phenylpropyl)-p-tert.-amylaniline
- 20 N - (p - benzoylacetaminobenzenesulphonyl) - N - benzyl-m-toluidine

If faster negative-type emulsions are used, a blue light absorber between the blue-sensitive emulsion and the green- and red-sensitive emulsions would be necessary. Colloidal silver cannot be used for this purpose, but a yellow dye filter layer such as described in Saunders et al. U.S. application Serial No. 476,066 would be suitable.

30 The nucleating agent for dissolved silver salts, which nucleating agent is incorporated in the emulsion layer, comprises colloidal metals, e.g., silver, metallic sulfides, e.g., silver sulfide, colloidal sulfur, or fogged silver halide.

The acceptor for oxidized developer is a non-diffusing reducing agent such as amyl hydroquinone, lauryl hydroquinone, 2,5-di-sec. octyl hydroquinone, 2,5-didodecyl hydroquinone, dodecyl catechol, 2,5-di-n-octyl hydroquinone, 2,6-di-n-octyl hydroquinone, and others.

The following example illustrates our invention:

### Red-sensitive layer

The following were mixed and coated over 2160 square feet of cellulose ester film support:

|    |                                                                                                                     |       |        |
|----|---------------------------------------------------------------------------------------------------------------------|-------|--------|
| 45 | One mole of red-sensitive gelatino-silver chlorobromide emulsion containing 80 grams of gelatin (80% chloride)----- | grams | 1360   |
|    | 10% gelatin solution-----                                                                                           | do    | 8160   |
| 50 | Colloidal silver dispersion 33 grams in 72.5 grams of gelatin and water to-----                                     | grams | 1160   |
|    | Cyan coupler dispersion-----                                                                                        | do    | 1545   |
|    | 2,5-di-sec. octylhydroquinone dispersion-----                                                                       | do    | 618    |
|    | Saponin 7.5% solution-----                                                                                          | cc    | 820    |
| 55 | Mucochloric acid 2.64% solution-----                                                                                | cc    | 214    |
|    | Water to -----                                                                                                      | grams | 24,500 |

### Green-sensitive layer

60 The following were mixed and coated over the red-sensitive emulsion covering an area of 2160 square feet:

|    |                                                                                                                       |       |        |
|----|-----------------------------------------------------------------------------------------------------------------------|-------|--------|
| 65 | One mole of green-sensitive gelatino-silver chlorobromide emulsion containing 80 grams of gelatin (80% chloride)----- | grams | 1410   |
|    | 10% gelatin solution-----                                                                                             | do    | 8160   |
|    | Colloidal silver dispersion (as above)-----                                                                           | do    | 1160   |
|    | Magenta coupler dispersion-----                                                                                       | do    | 1545   |
|    | 2,5-di-sec. octyl hydroquinone dispersion-----                                                                        | do    | 618    |
|    | Saponin 7.5% solution-----                                                                                            | cc    | 820    |
| 70 | Mucochloric acid 2.64% solution-----                                                                                  | cc    | 214    |
|    | Water to -----                                                                                                        | grams | 24,500 |

## Blue-sensitive layer

The following were mixed and coated over the green-sensitive emulsion covering an area of 1440 square feet:

|                                                                                                            |       |        |
|------------------------------------------------------------------------------------------------------------|-------|--------|
| One mole of high speed gelatino-silver chloro-bromide emulsion containing 80 grams gel (2% chloride) ----- | grams | 999    |
| 10% gelatin solution -----                                                                                 | do    | 4,850  |
| Colloidal silver dispersion containing 27.6 grams in 60.5 grams of gelatin and water to a total of -----   | grams | 969    |
| Yellow coupler dispersion -----                                                                            | do    | 1,285  |
| 2,5-di-sec. octyl hydroquinone dispersion -----                                                            | do    | 555    |
| Saponin 7.5% solution -----                                                                                | cc    | 550    |
| Mucochloric acid 2.64% solution -----                                                                      | cc    | 143    |
| Water to -----                                                                                             | grams | 16,400 |

The above dispersions were prepared as follows:

## 2,5-di-sec. octyl hydroquinone dispersion

3.5 grams of the di-octyl hydroquinone were dissolved in 105 cc. of dibutylphthalate and the solution dispersed in a mixture of 250 grams of 10% gelatin solution and 50 cc. of 5% Alkanol B solution. The dispersion was run through a colloid mill and brought to a final weight of 500 grams by adding water.

## Coupler dispersions

The coupler dispersions were prepared by dispersing a solution composed of 56 grams of coupler and 128 cc. of dibutylphthalate in a mixture of 260 grams of 10% gelatin solution and 50 cc. of 5% Alkanol B solution. This dispersion was run through a colloid mill several times and finally adjusted to a total weight of 500 grams by adding water.

The cyan coupler was 2-(diamylphenoxy acetamino)-4,6-dichloro-5-methyl phenol. The magenta coupler was 1-(2,4,6-trichlorophenyl)-3-[3'-(2",4"-di-tert. amylphenoxy acetamido)-benzamido]-5-pyrazolone. The yellow coupler was N-(4-benzoylacet-aminobenzene sulfonyl)-N-( $\gamma$ -phenyl propyl)-p-toluidine.

Exposed strips of this three-layer coating were processed as follows:

Film was developed for 5 to 10 minutes at 68° F. in a developer of the following composition:

|                                      |       |
|--------------------------------------|-------|
|                                      | Grams |
| N-methyl-p-aminophenol sulfate ----- | 6     |
| Hydroquinone -----                   | 10    |
| Sodium sulfite -----                 | 50    |
| Sodium carbonate -----               | 30    |
| Potassium bromide -----              | 5     |
| Water to 1 liter.                    |       |

After a short acetic acid stop bath and water wash the film was then developed in a color developer of the following composition:

|                                          |       |
|------------------------------------------|-------|
|                                          | Grams |
| 2-amino-5-diethylamino toluene HC1 ----- | 2     |
| Sodium sulfite -----                     | 2     |
| Sodium carbonate -----                   | 20    |
| Potassium bromide -----                  | 2     |
| Potassium thiocyanate -----              | 2     |
| Water to 1 liter.                        |       |

After an acetic acid stop bath and water wash the film was then treated in the usual ferricyanide and bromide bleach bath, washed, fixed with hypo and washed. These

processed strips showed excellent reversal, low stain and good color separation.

In place of potassium thiocyanate other silver halide solvents such as hypo, ammonium sulfite, etc. can be used in the color development.

In the accompanying drawing which shows a sectional view of a film coated according to our invention, 10 is a support of film base, glass, synthetic resin or other suitable material on which is coated the successive emulsion layers 11, 12 and 13, sensitive respectively to red, green and blue light and containing the appropriate color coupler as described above, a nucleating agent such as colloidal silver and a non-diffusing reducing agent or acceptor for oxidized developer.

It will be understood that various changes may be made in the process and materials described above and that our invention is to be construed as limited only by the scope of the appended claims.

What we claim is:

1. A multilayer reversal color material comprising a support having thereon a red-sensitive gelatino-silver halide emulsion layer containing a non-diffusing cyan color-forming compound, a green-sensitive gelatino-silver halide emulsion layer containing a magenta color-forming compound, and a blue-sensitive gelatino-silver halide emulsion layer containing a yellow color-forming compound, said emulsion layers being immediately superposed on each other and said color-forming compounds being capable of coupling with the oxidation product of a primary aromatic amino color developer, each of said emulsion layers containing a nucleating agent selected from the class consisting of colloidal silver, silver sulfide, colloidal sulfur, and fogged silver halide for catalyzing the precipitation of dissolved silver salts and a non-diffusing reducing agent for oxidized developer, said non-diffusing reducing agent being selected from the class consisting of higher alkyl hydroquinones containing at least 5 carbon atoms in the alkyl radical and higher alkyl catechols containing at least 5 carbon atoms in the alkyl radical.

2. A multilayer reversal color material comprising a support having thereon a red-sensitive gelatino-silver halide emulsion layer containing a non-diffusing cyan color-forming compound, a green-sensitive gelatino-silver halide emulsion layer containing a magenta color-forming compound, and a blue-sensitive gelatino-silver halide emulsion layer containing a yellow color-forming compound, said emulsion layers being immediately superposed on each other and said color-forming compounds being capable of coupling with the oxidation product of a primary aromatic amino color developer, each of said emulsion layers containing colloidal silver and 2,5-di-sec.-octyl hydroquinone.

## References Cited in the file of this patent

## UNITED STATES PATENTS

|           |                       |               |
|-----------|-----------------------|---------------|
| 2,306,410 | Schinzel -----        | Dec. 29, 1942 |
| 2,403,721 | Jelley et al. -----   | July 9, 1946  |
| 2,673,800 | Meeussen et al. ----- | Mar. 30, 1954 |
| 2,712,995 | Weyde -----           | July 12, 1955 |
| 2,725,298 | Yutzy et al. -----    | Nov. 29, 1955 |
| 2,740,717 | Yutzy et al. -----    | Apr. 3, 1956  |

## OTHER REFERENCES

Mees: The Theory of the Photographic Practice, pages 87-88, The MacMillan Co., New York, 1954.